

1

2,701,811

REACTION PRODUCT OF ZINC OXIDE AND  
ALDONIC ACIDS

Allan E. Chester, Highland Park, Ill., assignor to Poor & Company, Chicago, Ill., a corporation of Delaware

No Drawing. Application August 19, 1950,  
Serial No. 180,500

2 Claims. (Cl. 260—429)

This invention relates to new and useful organic compounds and more particularly to the reaction products of aldonic acids with zinc oxide and to a method for the preparation thereof.

This application is a continuation-in-part of my co-pending application, Serial No. 34,127, filed June 19, 1948, which matured into United States Patent 2,576,997.

It is an object of the invention to produce water soluble organic compounds which are substantially free from impurities.

Another object of the invention is to produce new and useful reaction products of zinc oxide and aldonic acids. A further object of the invention is the provision of a new and improved method for preparing compounds of the type referred to above.

Other objects and advantages of the invention will appear in the following disclosure.

In accordance with the invention it has been found that new and useful products are obtained by reacting zinc oxide with aldonic acids. The preferred products are acid soluble and are suitable for use in a number of ways, especially in electroplating baths and particularly in acid zinc electroplating baths. The preferred use of the products in electroplating baths is more fully described in my above-identified copending application.

The aldonic acids employed in this invention are derived from aldose sugars by oxidation thereof. A number of suitable aldonic acids are known, e. g., gluconic, mannonic, galactonic and arabinic acids. All of the aldonic acids exist in alpha and beta lactone forms. Gluconic acid is preferred for the practice of this invention because it is more cheaply and readily available than the other aldonic acids. The invention is not, however, limited to the use of gluconic acid.

The gluconic acid employed in the practice of the invention exists in several forms and the invention contemplates the use of one or more of these forms or mixtures thereof including mixtures of the lactone forms. Commercial gluconic acid is available as a 50% aqueous solution of approximately 99% gluconic acid and 1% glucose. The presence of the glucose is undesirable because it tends to build up in a plating bath and thereby cause gumminess and stickiness in the bath.

The zinc gluconate prepared according to this invention is substantially free of glucose. It is prepared by heating a commercial 50% gluconic acid solution to about 120° F. for a time sufficiently long to melt any crystalline lactone that might be present. Then one mole of lead free zinc oxide is added for every two moles of gluconic acid present. The mixture is heated to 170° F. with agitation and held for ten minutes or until solution of the ingredients is complete. The resultant product is cooled to 120° F. in the liquid phase and poured into large stoneware ves-

2

sels and cooled until a waxy solid forms along with some supernatant liquor. The liquor is mainly glucose and water and is removed from the solid by filtration. The residue is placed in drying trays where it may be washed with ice water to remove traces of residual glucose. The product is then dried by heating at temperatures below 250° F. until it becomes dry and hard, after which it is ground in a hammer mill or other suitable means. The resultant product is stable and non-sticky.

10 The foregoing description of the preparation of zinc gluconate is adaptable to the preparation of zinc aldonates in general by heating together one mole of zinc oxide with approximately two moles of any of the aldonic acids.

The zinc aldonate reaction product may be added to acid zinc electroplating baths according to the method outlined in my previously identified copending application in small amounts to effect a considerable increase in the brightness of the electroplated zinc plate. No further chemical treatment of the plates is necessary to bring out the brightness thereof. The reaction product also has a pronounced anti-burn effect when added to zinc plating baths.

15 It should be noted that glucose, when added alone to acid zinc plating baths, will not produce bright zinc plates. 20 Glucose or other aldoses therefore are in no sense the equivalent of gluconic or other aldonic acids or the reaction products thereof with zinc oxide for the purpose of the present invention.

The invention is hereby claimed as follows:

30 1. A process of preparing an acid soluble zinc gluconate which comprises heating a 50% by weight aqueous solution of approximately 99% gluconic acid and 1% glucose to a temperature of about 120° F. for a time sufficiently long to melt any crystalline lactone, then adding to said solution one mole of lead free zinc oxide for every two moles of gluconic acid present in the solution, heating the resultant mixture to 170° F. with agitation until solution of the added ingredients is complete, cooling the resultant product to about 120° F. in the liquid phase, pouring the resultant liquid into vessels and further cooling until a waxy solid forms along with some supernatant liquor, removing the supernatant liquor, washing the residual solid with water and drying the washed solid product at temperatures below 250° F.

45 2. A process of preparing an acid soluble zinc gluconate which comprises heating an aqueous solution of gluconic acid containing minor amounts of glucose to a temperature and for a time sufficiently long to melt any crystalline lactone, then adding to said solution approximately one mole of lead free zinc oxide for every two moles of gluconic acid present in the solution, heating the resultant mixture with agitation until solution of the added ingredients is complete, cooling the resultant product in the liquid phase, pouring the resultant liquid into vessels, further cooling until a waxy solid forms along with some supernatant liquor, removing the supernatant liquor and drying the solid product.

References Cited in the file of this patent

UNITED STATES PATENTS

1,893,872 Schmidt \_\_\_\_\_ Jan. 10, 1933

OTHER REFERENCES

65 Ber., vol. 49, pages 720-21, Jour. of Chem. Soc. (London), 1880, pages 795-6.

Beilstein, vol. 3, 4th edition, 1921, page 544.